

June 21, 1938.

W. ESPE

2,121,589

EMISSIVE INCANDESCENT CATHODE

Filed May 1, 1935

Fig. 1.



Fig. 2.



Fig. 3.



WITNESSES:

*E.G. Leiding*  
*R.W. Bailey*

INVENTOR

*Werner Espe.*

BY

*F.W. Lyle*,  
ATTORNEY

## UNITED STATES PATENT OFFICE

2,121,589

## EMISSIVE INCANDESCENT CATHODE

Werner Espe, Berlin-Siemensstadt, Germany,  
assignor to Westinghouse Electric & Manufacturing Company, East Pittsburgh, Pa., a corporation of Pennsylvania

Application May 1, 1935, Serial No. 19,233  
In Germany June 28, 1934

2 Claims. (Cl. 250—27.5)

My invention relates to cathodes and it has particular relation to cathodes having a vaporizable electron emitting substance.

It is an object of my invention to provide a cathode having a very long life. More specifically stated it is an object of my invention to provide a cathode in which a reservoir of electron emitting material is contained within a porous metallic mass, whose pores are also permeated with the electron emitting material.

Other objects of my invention will become evident from the following detailed description, taken in conjunction with the accompanying drawing, in which:

15 Figure 1 is a view, partly in elevation and partly in section, of a tube incorporating my invention.

Fig. 2 is a modification of the cathode structure illustrated in Fig. 1, and

20 Fig. 3 is a still further modification of the cathode structure of Fig. 1.

Incandescent cathodes manufactured up to the present time have the disadvantage that their life is comparatively short, since the emissive material quickly loses its emissive power. The cathodes have been coated rather heavily to increase the life of this type of cathode. It has been found, however, that this thick outer surface has a comparatively large internal resistance, and local overheating results with the possibility of eruptions from the surface.

According to my invention, I extend the life of a cathode by utilizing a porous metallic mass permeated with electron emissive material, and 35 I preferably provide a pocket within this mass having an additional reservoir of electron emitting material.

In Fig. 1 is disclosed the container 10 having an anode 11 and preferably a grid 12 therein of well-known construction. The cathode structure 13 preferably comprises a mass 14. This mass is preferably a sintered porous body composed of numerous fine angular metallic particles, and is 45 preferably permeated with vapor of an emissive material or has its pores filled with an emissive material vaporizable by heat. This cathode body is comparatively thick and may be, as shown, a cylindrical block, the height of which may be substantially equivalent to its cross-section.

50 While other materials may be used, I prefer to construct the body 14 of tungsten.

One method of constructing this body may be as follows. Barium azide ( $Ba(N_3)_2$ ) and tungsten in pulverized condition are mixed and 55 formed into a body under high pressure. The

body thus contains barium throughout, and when the body is heated, the nitrogen evaporates in such a manner that a mixture of barium and tungsten remains. The barium serves as emissive material and permeates the whole body. 5

Tungsten powder may also be heated to an incandescent temperature approximately 700° to 800° and then sintered. Oxides are formed on its surface. The powder may then be compressed under high pressure temperatures that 10 are lower than the decomposition temperature of the oxide and the body formed. Channels can be provided in the outer portion of the body, and these channels or pores permeated with an emissive material penetrating deep into the inner portion. As the emission takes place from the outer surface, the material distributed throughout the inner part of the body replenishes the vaporized portion from the surface. 15

These bodies, while being formed, could be 20 dipped into an electron emitting substance, such as barium or barium compound. Many materials which are now well known are capable of use in these cathodes, but the material selected should be one that can be capably absorbed by 25 the body. The body may be constructed of other sintered materials other than tungsten, and it is also conceivable that the sintering of the cathode body may be omitted. The body which is to absorb the emissive material should, however, 30 be filled with numerous small spaces. The oxidizing of the surface of these pores aids in absorbing and holding the emissive material.

I also prefer to provide a pocket or recess 35 in the cathode body, and to provide a reservoir 16 of vaporizable electron emissive material therein. This material may be an alkaline earth, as for example barium, or an alkali, such as potassium or sodium. The barium vapor, if barium is used, diffuses through the whole body 40 and produces on the walls of the recess and in the recess a precipitation which serves as the emissive material. If sintered tungsten powder is used as the cathode body material, then if the surface of the tungsten particles are slightly 45 oxidized to have a tungsten oxide of a low order formed on the outer surface, a better adherence of the emissive material thereto is attained. If tungsten particles having a basic oxide on their surface are utilized, then these 50 tungsten particles can be formed by subjecting them to pressure at high temperatures below 900° C.

It is also possible to provide a cathode body by mixing aluminum with barium oxide and 55

forming it under pressure. This body is heated to approximately 1000° C. and the barium is released and the aluminum transformed into aluminum oxide.

- 5     In order to provide an efficient means for vaporizing the electron emitting material, I preferably place the cathode body 14 on a metallic plate 17. The plate 17 has adjacent thereto a heating body, such as the filament 18. The plate 17 may take the form of a part of the casing wall and be sealed to the tube as at 19. A connection 20 is made from one of the heating leads 21 to the metal plate 17, and in this way the plate 17 forms a cathode connection to the cathode body 14. A separate lead-in connection may be made to the cathode, if desired. Any suitable support and closure member for the filament 18, such as the insulating plate 22, may be provided.
- 10    The material of the metal plate 17 may be of copper or of other vacuum-tight metals. In case a separate lead-in to the cathode is desired, then the portion 17 may be of insulating material or may be replaced by a cathode lead supported from the usual press.
- 15    Fig. 2 discloses a modification of the cathode structure, in which the cathode body 14 has a recess 15 formed therein with a reservoir of electron emitting material 16. This recess 15 is preferably threaded, and a closure body 24, composed of sintered material, is threaded into the threads 25. This closure member 24 is used as a support and as a connecting element. The closure body 24 may have, if desired, a heating element or filament 26 disposed therein or only a single
- 20    cathode connection thereto.
- 25    Fig. 3 discloses a still further modification in

which channels 38 are formed in the outer surface or portion of the body and a heating element 31 placed in these channels. The pores of the body 14 will act as wicks of electron emitting material heated at their outer ends.

From the foregoing description, it is apparent that the porous body 14 may have electron emitting material or vapor permeated throughout its construction. As the device is operated, this electron emitting material is gradually drawn out through the porous structure of this body. The electron emitting material 16 and the recess replenishes the part used up and provides a very much longer life for these indirectly heated cathodes over the structure of the prior art.

10    Although I have shown and described certain specific embodiments of my invention, I am fully aware that many modifications thereof are possible. My invention, therefore, is not to be restricted, except insofar as is necessitated by the prior art.

15    I claim as my invention:

1. A cathode structure comprising a mass of sintered tungsten particles having pores therein, portions of the surface of said pores being coated 25 with an oxide of said metal and an electron emitting substance on said oxide and a pocket in said mass having a reservoir of said electron emitting substance.

2. A cathode structure comprising a porous 30 mass of sintered tungsten having a pocket therein, an electron-emitting vaporizable substance in said pocket, and means for vaporizing said substance.

WERNER ESPE. 35